

March 31, 1936.

T. V. FOWLER, JR

**2,035,699**

## METHOD AND APPARATUS FOR ROASTING ORES

Filed Dec. 19, 1931



INVENTOR  
T. V. Fowler, Jr.  
BY *Fowler Silsby*  
ATTORNEY

## UNITED STATES PATENT OFFICE

2,035,699

METHOD AND APPARATUS FOR  
ROASTING ORES

Theodore V. Fowler, Jr., Pelham, N. Y., assignor  
to General Chemical Company, New York,  
N. Y., a corporation of New York

Application December 19, 1931, Serial No. 582,082

20 Claims. (Cl. 75—60)

This invention relates to roasting sulfide ores, and is directed more particularly to a method and apparatus for roasting finely divided sulfide ores of the type customarily requiring extraneous heat to effect substantially complete desulfurization. One particular application of the invention lies in the roasting of zinc sulfides, such as finely divided zinc sulfide flotation concentrates. Broadly speaking, the invention contemplates a method including the preliminary phases of bed roasting with respect to the initial drying of the ore and heating the same to the ignition temperature, together with the principles of suspension roasting.

Bed roasting and suspension roasting of sulfide ores are known in the art. Bed roasting of finely divided sulfide ores has been widely practiced, for example, in the well known Herreshoff roasters. However, with respect to certain types of sulfide ores, such as zinc sulfides, and iron sulfides such as pyrrhotite, which contain comparatively small quantities of sulfur, difficulty in obtaining a good roast is often experienced because of insufficient available heat and it is often necessary in order to obtain reasonably satisfactory results to supply heat from extraneous sources to complete the roasting operation. Hence, it has been usual to carry out the roasting of zinc sulfides in furnaces equipped with muffled hearths in which producer or other combustible gas is burned for the purpose of supplying the required additional amounts of heat. Muffled hearth furnaces are themselves expensive to build, and the construction and upkeep of gas producers are large items of expense. A further disadvantage encountered in the roasting of zinc ores in hearth furnaces is that although high temperatures are desirable in the final stages to complete desulfurization, such high temperatures are not ordinarily obtainable without the supply of extraneous heat, and when extraneous heat is supplied to effect complete desulfurization the destructive effects on the rabbler mechanism become pronounced thus shortening the life of the roasting equipment and increasing production costs.

To overcome many of the difficulties of hearth roasting arising chiefly out of expensive equipment, suspension roasting has been proposed. However, when working with zinc sulfides the problem of supplying the additional heat again arises. Hence, it has been suggested to preheat the air used to form the gaseous suspension and support combustion, and to preheat the ore, or preheat both air and ore, the purpose being to raise the temperature of the ore to such an extent

that on introduction of the suspension into the combustion chamber, the ore is heated to approximately the ignition point. In practice, however, such preheating to raise the temperature of the ore to the ignition point has not been obtainable economically. Preheating the air has not been particularly successful, since the contact of the ore and air prior to the introduction of the suspension in the roasting chamber is so brief that the ore is not sufficiently heated. Preheating the ore raises a most important difficulty in providing suitable apparatus for conveying ores heated to temperatures in the neighborhood of 1000° F. or above, and for forming a gaseous suspension of such comparatively hot ore in air in a suitable mixing nozzle. Hence, the principal disadvantage in desulfurizing ores such as zinc sulfides in bed roasting is an incomplete roast, and with respect to suspension roasting, the difficulty lies in preheating the ore sufficiently so that ignition will ensue immediately following the introduction of the suspension in the roasting chamber.

The principal object of the present invention lies in the provision of a method and apparatus for suspension roasting of sulfide ores whereby the preheating of the ore to the ignition temperature on introduction into the roasting chamber is assured. According to the invention, the finely divided ore is subjected to preheating in an operation embodying the preliminary phases of bed roasting with respect to the initial drying of the ore and raising the temperature of the same to the ignition point. Such preheating is preferably carried out in an atmosphere of the hot gaseous products of combustion of the final suspension roasting. The ore, heated in this manner to, or substantially to, the ignition temperature, is fed into a roasting chamber preferably so that ignition of the ore takes place substantially immediately upon introduction of the ore into the roasting chamber, and combustion of the ore proceeds in a suspension of the ore in oxidizing gas in the roasting chamber. The invention is of particular value in the roasting of ores which customarily do or may require the application of extraneous heat to accomplish complete roasting.

Further objects of the invention and advantages thereof will appear from the following description taken in connection with the accompanying drawing illustrating partly in section and partly in elevation one embodiment of a roasting furnace particularly adapted for carrying out the invention.

Referring to the drawing, the apparatus includes principally a shaft roaster and a multi-hearth heater indicated generally by the reference numerals 10 and 11. The shaft roaster comprises a vertically elongated, preferably cylindrical combustion chamber 12 within a steel shell 13 lined with refractory material 14. The shaft roaster is supported by a frame 15, and suitable brickwork 16. The lower end of the combustion chamber is cone-shaped, forming a cinder pit 18 discharging into a cinder outlet 19 equipped with any approved form of gate. The shaft roaster is held in place laterally by structural framework 21. Spaced about the circumference 15 of the combustion chamber are air inlets 22. The discharge ends of the inlet passages are horizontally elongated, as indicated at 23, so as to cause introduction of air or other oxidizing gas into the combustion chamber in the form of 20 a series of more or less flat sheets. Any required number of inlets 22 may be provided at desirable vertical intervals. In the embodiment of the invention disclosed three sets are illustrated. Air is supplied to the inlets 22 through 25 bustle pipes 25, the inlets 26 of which open into an air inlet main 27.

The hearth heater 11 is positioned directly above the shaft roaster and rests upon a platform 30, the weight of the hearth heater and 30 associated mechanism being carried by the structural framework 21. The hearth heater comprises a heating chamber, indicated generally by the reference numeral 31, formed by vertical cylindrical walls 32, the drying deck 33 and the 35 lowermost hearth 34. The heater includes additional intermediate hearths 36 and 37. Ore inlets 38 extend through drying deck 33 adjacent walls 32 and openings 40 pass through hearth 37 around the periphery thereof. Hearth 36 is provided with a central ore and gas passage 41. The lowermost hearth 34 serves as the upper 40 end of the combustion chamber 12 of the shaft roaster, and includes a centrally disposed passage 43, and a plurality of openings 44 passing through 45 the hearth 34 intermediate the periphery of the passage 43 and the inner surface of the refractory lining 14 of the shaft roaster.

The rabbling mechanism for the hearths is of the general construction employed in the well 50 known Herreshoff roaster, and hence need not be described in detail. The rotatable shaft 46, having rabble arms 47, is mounted in bearings 48 and 49, the weight of the rabbling mechanism being transmitted to the framework through cross-member 50 and bearing 49. Shaft 46 has therein a longitudinal conduit 52 extending to bearing 48, and through which cooling air is passed into the rabble arms. The arrangement is such that the cooling air leaves the rabbling 55 arms 47 and the annular passage 55 by way of chamber 56 arranged in any suitable manner so as to permit rotation of the shaft 46 and conduit 52. Ore from a hopper 57 is fed intermittently onto the drying deck 33 by a sweep fixed to shaft 46. The ore supply in hopper 57 may be maintained by a conveyor not shown.

The gaseous products of the entire roasting 70 operation leave the apparatus through the gas outlet 60 in the upper end of the heating chamber 31, and pass through conduit 61 into a dust separator indicated generally by reference numeral 62. The latter may be of any desired construction, but is preferably a multi-cone type separator, having a plurality of gas-tight partitions 63 and constructed so as to permit pre-

heating of the air introduced into the shaft roaster through conduit 27. Gas from conduit 61 enters the chamber 64 and passes downwardly into a cone 65 in which dust settles out of the gas stream, the gas rising into chamber 67 through a cone 68. The dust free gases are then withdrawn from the apparatus through pipe 69, and utilized as desired, for example in the manufacture of sulfuric acid. Dust separated from the gas stream in cones 65 drops into the dust 10 discharge pipes 70 provided with suitable air locks 71.

Air for use both in the roasting operation and as a cooling medium in the rabbling mechanism is supplied through an air inlet 73. Part of the 15 air flows through the pipe 74 into the central conduit 52 in the shaft 46, and another part is passed through chamber 75, thus serving to cool the lower bearing of shaft 46. Air for the entire roasting operation is preheated by circulating 20 the same around cones 65 in chamber 76, and is then conducted into combustion chamber 12 through pipe 27. A by-pass 77, controlled by valve 78, is disposed between the upper end of chamber 12 and the outlet conduit 61 to facilitate 25 control of the quantity of hot gases passing through heating chamber 31 thus permitting regulation of the temperature therein. The degree of preheating of the air entering chamber 12 may be regulated by valve-controlled by-pass 80. 30

The roasting operation is carried out substantially as follows: Finely divided sulfide ore, such as zinc sulfide flotation concentrates, is continuously charged into hopper 57 from which small quantities are intermittently swept onto 35 the surface of the deck 33 on which excess moisture is removed from the ore by heat radiating from the roasting chamber 31. It will thus be seen that, according to the present method, comparatively wet concentrates may be employed, 40 whereas in prior suspension roasting, it has been necessary to provide additional apparatus for drying the ore before charging the same in the form of a gaseous suspension into the combustion chamber. As is known in the art, the plows on 45 the uppermost rabbling arm are so arranged as to slowly feed ore through the passages 38 to the hearth 36. Drying is furthered and pre-heating is commenced to some extent on the hearth 36 over which the ore is gradually worked 50 toward and discharged through the central opening 41 to the intermediate hearth 37. As the ore passes over the upper hearths, the temperature of the ore is gradually increased, until by the time the ore is discharged through passages 55 40 onto the lowermost hearth 34, preheating is well initiated, and the temperature of the ore approaches the ignition point. During the inward movement of the ore over lower hearth 34, the temperature is further raised, and when the 60 ore is discharged into the upper end of the shaft roaster through openings 43 and passages 44, the temperature of the ore is substantially at the ignition point, for example around 1400°-1600° F. It will be seen that on account of the particular 65 arrangement of central opening 43 and the several passages 44, the ore is fed from the hearth 34 into the shaft roaster in a shower resembling two concentric cylinders, thus facilitating the formation of a suspension of the ore in an oxidizing 70 gas in the shaft roaster.

Air in quantities necessary to supply oxygen for the entire roasting operation is introduced into the shaft roaster through the several inlets 22, and rises through chamber 12, countercurrent to 75

the downward passage of the burning ore. This upward movement of air effects the formation of a suspension of the finely divided ore, and further serves to retard sufficiently the descent of any 5 heavier particles of ore to facilitate complete desulfurization.

The temperature of the ore on the lower hearth 34 may be at or possibly slightly above the ignition temperature, and hence, combustion of the 10 ore particles takes place almost instantaneously upon the introduction of the ore into the upper end of the shaft roaster. Since ignition is immediately brought about, desulfurization proceeds rapidly, and is completed in the central zone of 15 chamber 12, considerably before the ore particles fall into the cinder pit 18. Accordingly, on account of the high temperatures easily attainable in shaft roasting, complete desulfurization is assured. The sulfur dioxide gases from the shaft 20 roaster, at temperatures around 1800-2000° F., enter the upper chamber 31 through the opening 43, pass successively over the hearths, and are withdrawn from the apparatus through conduit 61. During passage through chamber 31, the hot 25 gases are in direct contact with the ore on the several hearths, thus effecting drying and preliminary heating of the ore and positively raising the temperature thereof to about the ignition point. In the event that the temperature in 30 chamber 31 should become undesirably high, necessary quantities of hot gases from chamber 12 may be by-passed around chamber 31 through pipe 77 by suitable regulation of valve 78.

The advantages arising from the invention are 35 numerous. Primarily, the temperature of the ore on introduction into the roasting chamber 12 may be at or around the ignition point, so that combustion is instantaneously initiated. High finishing roasting temperatures are easily attainable in 40 the combustion chamber, with the result that the ore is completely desulfurized and no equipment having moving parts is damaged because of the high temperatures. Additional heat, beyond that generated in the roasting operation as a whole, is 45 not required. Wet ore or concentrates may be used at the start, thus avoiding the necessity of additional drying apparatus particularly where wet concentrates are employed. The necessity of handling hot preheated ore in specially designed 50 conveying apparatus is avoided. The invention further makes available, in the roasting of sulfide ores, such as zinc-sulfides, pyrrhotite, pyrites, etc., the full economic benefits of suspension roasting, and additionally assures heating of the 55 ore to ignition temperature just prior to introduction into the shaft roaster by reason of the preliminary direct contact of the ore and the highly heated effluent gases of the suspension roasting stage.

60 I claim:

1. The process of roasting finely divided sulfide ores which comprises heating the ore in a bed heating operation by feeding the ore in countercurrent flow with hot gaseous combustion products of a succeeding roasting operation, and then feeding the ore into a combustion chamber and roasting the ore in suspension in an oxidizing gas.
2. The process of roasting finely divided sulfide 70 ore which comprises agitating a bed of the ore while heating the ore in an atmosphere comprising the gaseous combustion products of a succeeding roasting stage to such extent that the temperature of the ore is raised substantially to the ignition point, and then feeding the ore into 75 the ignition point, and then feeding the ore into

a combustion chamber and roasting the ore in suspension in an oxidizing gas to substantially complete desulfurization.

3. The process for roasting finely divided metal sulfides in an operation involving a heating stage 5 and a roasting stage in which the sulfide fines are burned in an oxidizing gas which process comprises applying heat to the fines in the heating stage by causing hot gases from the succeeding roasting stage to flow in direct contact with said 10 fines whereby the latter are heated in an atmosphere comprising hot gases from the succeeding roasting operation, and then feeding the fines into a combustion zone constituting the roasting stage, roasting the fines in said zone while 15 in suspension in oxidizing gas to produce sulfur dioxide gases and oxide cinder, recovering sulfur dioxide gases from the roasting stage, and discharging cinder therefrom.

4. The process for roasting finely divided metal 20 sulfides in an operation involving a heating stage and a roasting stage in which the sulfide fines are burned in an oxidizing gas which process comprises maintaining a bed of fines in the heating stage, passing the fines forming the bed through 25 the heating stage while agitating the fines and heating the same in an atmosphere comprising hot gases from the succeeding roasting operation passing through the heating stage, and then feeding the fines into a combustion zone constituting 30 the roasting stage, roasting the fines in said zone while in suspension in oxidizing gas to produce sulfur dioxide gases and oxide cinder, recovering sulfur dioxide gases from the roasting stage, and discharging cinder therefrom.

5. The process of roasting finely divided sulfide 35 ores which comprises heating the ore by feeding the ore in countercurrent flow with hot gaseous combustion products of a succeeding roasting operation, and then feeding the ore into a combustion chamber and roasting the ore in suspension in an oxidizing gas.

6. The process of roasting finely divided sulfide ore which comprises heating a bed of the ore to 45 such extent that the temperature thereof is raised substantially to the ignition point, and then feeding the ore into a combustion chamber and roasting the ore therein to substantially complete desulfurization while maintaining the ore in suspension in an oxidizing 50 gas flowing countercurrent to the movement of the roasting ore.

7. The process of roasting finely divided sulfide 55 ore which comprises agitating a bed of the ore while heating the ore in an atmosphere comprising the gaseous combustion products of a succeeding roasting stage to such extent that the temperature of the ore is raised substantially to the ignition point, and then feeding the ore into a combustion chamber and roasting the ore therein to substantially complete desulfurization while 60 maintaining the ore in suspension in an oxidizing gas flowing countercurrent to the movement of the roasting ore.

8. The process of roasting finely divided zinc sulfide ore which comprises heating the ore in 65 a bed heating operation to such extent that the temperature of the ore is raised substantially to the ignition point, and then feeding the ore into a combustion chamber and roasting the ore therein to substantially complete desulfurization 70 while maintaining the ore in suspension in an oxidizing gas flowing countercurrent to the movement of the roasting ore.

9. The process of roasting finely divided zinc sulfide ore customarily requiring the application 75

of extraneous heat to effect substantially complete desulfurization which comprises heating the ore in a bed heating operation in an atmosphere comprising the gaseous combustion products of the succeeding roasting stage to such an extent that the temperature of the ore is raised substantially to the ignition point, and then feeding the ore into a combustion chamber and roasting the ore therein to substantially complete desulfurization while maintaining the ore in suspension in an oxidizing gas flowing countercurrent to the movement of the roasting ore.

10. Apparatus for roasting finely divided sulfide ore to effect substantially complete desulfurization which comprises means for agitating a bed of the ore while heating the same, means for effecting such heating in an atmosphere comprising gaseous combustion products of a succeeding roasting stage, a combustion chamber, means for then feeding the ore into the combustion chamber, and means for forming in the combustion chamber a suspension of the ore in an oxidizing gas, whereby the ore is roasted to substantially complete desulfurization.

11. Apparatus for roasting finely divided metal sulfide in suspension in an oxidizing gas comprising a vertically disposed roasting furnace comprising a sulfide fines heating chamber in the upper part of said furnace and a combustion chamber in the lower part of the furnace, a fines heating hearth in said heating chamber, means for maintaining on said hearth a bed of sulfide fines, means for causing said bed of fines to pass over said hearth while agitating the fines during passage of the same over said hearth, means including a connection between the combustion chamber and the heating chamber for flowing hot gases from the combustion chamber over the bed of fines during passage of the bed of fines through the heating chamber, whereby said fines are heated in an atmosphere comprising hot gases of a succeeding roasting operation, means for introducing fines after passage over said hearth into the combustion chamber and for forming therein a suspension of the fines in oxidizing gas whereby the fines are roasted to produce sulfur dioxide gases and oxide cinder, means for withdrawing sulfur dioxide gases from the combustion chamber, and means for discharging cinder therefrom.

12. Apparatus for roasting finely divided sulfide ore to effect substantially complete desulfurization which comprises means for agitating a bed of the ore while heating the same, means for effecting such heating in an atmosphere comprising gaseous combustion products of a succeeding roasting stage, a combustion chamber, means for then feeding the ore into the combustion chamber, and means for forming in the combustion chamber a suspension of the ore in an oxidizing atmosphere comprising means for passing through said chamber, counter to the movement of the ore, a current of oxidizing gas, whereby the ore is roasted to substantially complete desulfurization.

13. Apparatus for roasting ores comprising a heating bed, means for feeding ore to said bed, means for agitating ore on the bed while undergoing heating thereon, a combustion chamber, means for passing ore from the bed into the combustion chamber in the form of a shower, and means for passing through the chamber, counter to the movement of the ore therein, a stream of oxidizing gas, whereby the ore is roasted in the combustion chamber in gaseous suspension.

14. Apparatus for roasting ore comprising a chamber, a heating hearth in the chamber, means for feeding ore to the hearth, means for agitating ore on the hearth while undergoing heating thereon, a combustion chamber, means for passing ore from the hearth into the combustion chamber in the form of a shower, means for forming in the combustion chamber a suspension of the ore in an oxidizing gas, and means for conducting the gaseous products of combustion from the combustion chamber over the roasting hearth, whereby heat is imparted to the ore undergoing heating on the hearth, and the gaseous products of the entire roasting operation become intermingled.

15. Apparatus for roasting finely divided metal sulfide in suspension in an oxidizing gas comprising a vertically disposed roasting furnace comprising a sulfide fines heating chamber in the upper part of said furnace and a combustion chamber in the lower part of the furnace, a fines heating hearth in said heating chamber, means for maintaining on said hearth a bed of sulfide fines, means for causing said bed of fines to pass over said hearth while agitating the fines during passage of the same over said hearth, means including a connection between the combustion chamber and the heating chamber for flowing hot gases from the combustion chamber over the bed of fines during passage of the bed of fines through the heating chamber, whereby said fines are heated in an atmosphere comprising hot gases of a succeeding roasting operation, means for introducing fines after passage over said hearth into the combustion chamber and for forming therein a suspension of the fines in oxidizing gas, whereby the fines are roasted to produce sulfur dioxide gases and oxide cinder, means for heating said oxidizing gas prior to admission to said combustion chamber by heat generated in the roasting operation, means for withdrawing sulfur dioxide gases from the combustion chamber, and means for discharging cinder therefrom.

16. Apparatus for roasting ores comprising a vertically disposed shaft roaster having an opening at the upper end thereof, a heating hearth mounted above the shaft roaster, means for feeding ore to the hearth and means for agitating ore undergoing heating on the hearth, means for gradually feeding ore from the hearth into the upper end of the shaft roaster, and means for introducing oxidizing gas into the lower portion of the shaft roaster for forming a suspension of the ore in a counter current flow of oxidizing gas.

17. Apparatus for roasting ores comprising a vertically disposed shaft roaster having an opening at the upper end thereof, a chamber mounted directly above the shaft roaster, an outlet for the chamber positioned immediately above the opening in the shaft roaster, a plurality of heating hearths in said chamber, means for feeding ore to the uppermost of said hearths, means for gradually passing ore while agitating the same successively over the hearths, means for gradually discharging ore from the lowermost hearth into the upper end of the shaft roaster, and means for introducing oxidizing gas into the lower portion of the shaft roaster for forming a suspension of the ore in a counter current flow of oxidizing gas.

18. Apparatus for roasting ores comprising a vertically disposed shaft roaster having an opening at the upper end thereof, a chamber mounted directly above the shaft roaster, an outlet for

the chamber positioned immediately above the opening in the shaft roaster, a plurality of heating hearths in said chamber, means for feeding ore to the uppermost of said hearths, means for gradually passing ore while agitating the same successively over the hearths, means for gradually discharging ore from the lowermost hearth into the upper end of the shaft roaster in the form of a shower, means for passing upwardly through the shaft roaster a stream of oxidizing gas, whereby a suspension of the ore in the gas is formed, and means for passing the gaseous products of combustion of the shaft roaster through the hearth chamber, thereby imparting heat to the ore undergoing heating on the hearths, and mingling the gaseous products of the entire roasting operation.

19. The process of roasting finely divided zinc sulfide ore customarily requiring the application of extraneous heat to effect substantially complete desulfurization which comprises heating the ore in a bed heating operation in an atmosphere comprising the gaseous combustion products of the succeeding roasting stage to such an extent that the temperature of the ore is raised substantially to the ignition point, preheating an oxidizing gas, feeding the ore into a combustion chamber and roasting the ore therein to substantially complete desulfurization while maintaining the ore in suspension in said preheated

oxidizing gas flowing counter-current to the movement of the roasting ore.

20. Apparatus for roasting ores comprising a vertically disposed shaft roaster having an opening at the upper end thereof, a chamber mounted directly above the shaft roaster, an outlet for the chamber positioned immediately above the opening in the shaft roaster, a plurality of heating hearths in said chamber, means for feeding ore to the uppermost of said hearths, means for gradually passing ore while agitating the same successively over the hearths, means for gradually discharging ore from the lowermost hearth into the upper end of the shaft roaster in the form of a shower, a dust separator connected to the gas outlet of said chamber, means for passing oxidizing gas through said dust separator in heat exchange relation with hot combustion gases therein, whereby the oxidizing gas is preheated, means for passing upwardly through the shaft roaster a stream of preheated oxidizing gas, whereby a suspension of the ore in the gas is formed, and means for passing the gaseous products of combustion of the shaft roaster through the hearth chamber, thereby imparting heat to the ore undergoing heating on the hearths, and mingling the gaseous products of the entire roasting operation.

THEODORE V. FOWLER, JR. 30